

## UNITED STATES PATENT OFFICE

2,588,365

## METHOD OF RENDERING FABRICS WATER-REPELLENT AND PRODUCT RESULTING THEREFROM

Firth L. Dennett, Midland, Mich., assignor to Dow Corning Corporation, Midland, Mich., a corporation of Michigan

No Drawing. Application November 10, 1949,  
Serial No. 126,690

3 Claims. (Cl. 117—161)

1

This invention relates to a method of rendering fabrics water-repellent.

Siloxanes for treating fabrics to render them water-repellent have heretofore been known. "Mark-off" is a serious problem in connection with the heretofore known compositions. Mark-off is the appearance of lines when the treated fabric is folded or otherwise wrinkled. Mark-off appears especially in such fabrics as nylon, orlon and rayon of either viscose or acetate type. Heretofore, when the treated fabric was laundered or dry cleaned, a considerable amount of the oblique mark-off was noted.

It is an object of the present invention to provide a method whereby fabrics are rendered substantially water-repellent even after laundering and dry cleaning.

It is another object of the present invention to eliminate or materially reduce mark-off in fabrics rendered water-repellent, such as nylon, orlon and rayon of either viscose or acetate type.

It is a further object of the present invention to render fabrics water-repellent whereby the fabrics after treatment possess good "hand" and "drape," and are of better crease resistance.

In accord with the present invention, fabrics are rendered water-repellent by wetting the fabrics with a mixture of two organosiloxane polymers. The fabrics so wetted are then heated at a temperature ranging from 100° to 475° F. for a period of from 5 seconds to 1 hour.

The fabrics which may be treated in accord with the method of the present invention include fabrics of natural materials such as cotton, linen, silk or wool and fabrics of artificial material such as nylon, orlon and rayon of either viscose or acetate type.

One of the siloxane polymers used in the above stated mixture is a methylhydrogenpolysiloxane fluid which contains between 1.0 and 1.5 methyl radicals and between 0.75 and 1.25 hydrogen atoms bonded to silicon per silicon atom, there being a total of 2 to 2.25 methyl radicals and hydrogen atoms per silicon atom. Fluids of this type may be produced by the hydrolysis and condensation of  $\text{CH}_3\text{HSiCl}_2$  alone or by cohydrolyzing and condensing it with a chlorosilane, such as  $(\text{CH}_3)_3\text{SiCl}$ ;  $(\text{CH}_3)_2\text{HSiCl}$ ; and  $(\text{CH}_3)_2\text{SiCl}_2$ .

The other siloxane polymer used in the above stated mixture is a methylpolysiloxane fluid which contains between 2 and 2.1 methyl radicals per silicon atom and which has a viscosity of at least 1,000 centistokes and preferably less than 100,000 centistokes. Such fluids and their preparation have been described in the art and are now well-known commercially. They may be

2

produced by cohydrolyzing and condensing a mixture of methyl chlorosilanes of the general average formula  $(\text{CH}_3)_n\text{SiCl}_{4-n}$  where  $n$  has a value of from 2 to 2.1.

5 From 20 to 70 per cent by weight of the total mixture consists of the methylpolysiloxane and the remaining 80 to 30 per cent consists of the methylhydrogenpolysiloxane.

Catalysts may be added to the mixture of organosiloxanes, and the mixture then used to wet the fabric. Alternatively the fabric may be wetted with the organosiloxane mixture and the fabric dipped in a solution of the catalyst. Such catalysts include metallic salts such as sodium 10 bicarbonate, sodium aluminate and iron, cobalt, manganese, lead and zinc salts of carboxylic acids such as acetates, octoates and naphthenates.

This organosiloxane mixture may be applied 15 directly to the fabric. However, it is preferred to extend the organosiloxane mixture by diluting with a liquid hydrocarbon, chlorohydrocarbon, ether or alcohol, such as benzene, dioxane, ethanol or the like in order to minimize the 20 amount employed.

The organosiloxane mixture may likewise be extended by the preparation of an aqueous emulsion, which emulsion preferably contains an emulsifying agent decomposable by heating. The 25 quaternary ammonium halides are examples of such emulsifying agents. They are decomposed on heating for a brief period before the fabric is damaged by the heating. Examples of such halides are the alkylarylammonium chlorides, such as trimethylbenzylammonium chloride and hexadecyldimethylbenzylammonium chloride. If desired, the siloxane mixture may be thinned with any of the above indicated solvents in order to facilitate emulsification. After emulsification, the solvent may be removed under vacuum, if 30 desired.

Emulsions of methylhydrogenpolysiloxanes frequently liberate hydrogen upon standing. In order to avoid this effect, it is accordingly desirable to add an organic acid such as acetic acid to the emulsion in order to inhibit the evolution of hydrogen. The quaternary ammonium salts function well as emulsifying agents in such acid 35 systems.

The siloxane mixture either straight or as a solution or emulsion may be applied to the fabric in any appropriate manner. Thus, the fabric may be dipped in the mixture. The mixture may be applied to the fabric by the use of conventional equipment such as a padder or quetch.

## 3

The fabric may then be dried to remove water or solvent.

The material should be applied to the fabric in such amount that there is between 1 and 5 per cent of the organosiloxane mixture based upon the weight of the fabric.

The fabric is then heated to between 100° and 475° F. for from 5 seconds to 1 hour. This heating effects liberation of a major portion of the hydrogen which is bonded to the silicon in the dimethylhydrogenpolysiloxane. The decomposition product is polymerized to an insoluble polymer in the fabric, whereby the fabric is rendered permanently hydrophobic. When a heat decomposable emulsifying agent is employed, it is also decomposed during this heating.

The present invention is of particular importance in the hydrophobing of nylon and acetate rayon. In manufacturing filaments of these materials, the filaments are extruded in a molten state and the extrusion stretched while soft.

This results in a strain in the filaments. Frequently the fabrics are woven without the strain in the filaments being relaxed. Such a fabric may be wetted with a siloxane in accord with this invention. After wetting, the fabric is contacted with a hot surface at a temperature of 400° to 475° F. for from 5 to 80 seconds. This heat treatment serves a dual purpose, first, to set the siloxane polymer and second, to effect relaxation of the filament. The use of the siloxane improves the "ironability" of the fabric, since the coated fabric does not adhere to the iron nor do the fibers cohere even when slightly softened.

Fabrics treated in accord herewith are substantially water-repellent both after laundering and after dry cleaning. The contact angle between a drop of water and the surface of a fabric so treated is about 110°. Treated fabrics of cotton, linen, wool, nylon, orlon and rayon are soft to the touch and have a good hand. Nylon, orlon and rayon fabrics so treated have a reduced tendency to show mark-off.

The following polysiloxanes were prepared:

A mixture of 9.3 parts by weight of decamethyltetrasiloxane and 735 parts of octamethylcyclotetrasiloxane was prepared. To this mixture there were added .56 part of KOH. This mixture was then heated at 160° C. for 8 hours. The mixture was then cooled to about 100° C. and CO<sub>2</sub> in the form of Dry Ice was added over a period of 30 minutes. This mixture was then filtered and flash distilled to 250° C. at 1 mm. pressure. There were obtained 625 parts of a trimethylsiloxy end-blocked dimethylpolysiloxane fluid having a viscosity of 1,000 centistokes, which is referred to as product I in the examples.

A mixture was prepared of 1.5 parts by weight of decamethyltetrasiloxane and 735 parts of octamethylcyclotetrasiloxane. To this mixture there were then added .56 part of KOH. This mixture was then agitated and heated at 160° C. for 8 hours. The mixture was then cooled to about 100° C. and CO<sub>2</sub> in the form of Dry Ice added over a period of 30 minutes. The mixture was then filtered and flash distilled to 250° C. at 1 mm. pressure. There were obtained 630 parts of a trimethylsiloxy end-blocked dimethylpolysiloxane fluid having a viscosity of 12,500 centistokes, which is referred to as product II in the examples.

A mixture was prepared of 1.2 parts by weight of decamethyltetrasiloxane and 735 parts of octamethylcyclotetrasiloxane. To this mixture there was then added .56 part of KOH. The mixture was then agitated and heated at 160° C. for 75

## 4

8 hours. The mixture was then cooled to 100° C. and CO<sub>2</sub> in the form of Dry Ice added over a period of 30 minutes. The mixture was then filtered and flash distilled to 250° C. at 1 mm. pressure. There were thereby obtained 620 parts of a trimethylsiloxy end-blocked dimethylpolysiloxane having a viscosity of 30,000 centistokes, which is referred to as product III in the examples.

A mixture of 1,000 parts of CH<sub>3</sub>HSiCl<sub>2</sub> and 51.5 parts of (CH<sub>3</sub>)<sub>3</sub>SiCl was added to 750 parts of benzene. This mixture was then cooled to 20° C. To this mixture 675 parts of isopropyl alcohol were added over a period of 10 minutes and then 783 parts of water were added over a period of 1 hour, whereby to effect hydrolysis. An additional 750 parts of benzene were then added to the reaction mixture. The product was washed six times with water and strip distilled at 3 mm. pressure to 115° C. to remove the benzene and the lower boiling products. There were obtained 475 parts of a trimethylsiloxy end-blocked dimethylhydrogenpolysiloxane, which is referred to as product IV in the examples.

In the following examples, which are illustrative only, the "spray rating" was determined by standard test method 22-41 of the American Association of Textile Chemists and Colorists.

## Example 1

A mixture was prepared of 24 parts by weight of product IV and 6 parts of product I. To this siloxane mixture there were added 3 parts of hexadecyldimethylbenzylammonium chloride and 0.1049 part of acetic acid. The resulting mixture was then emulsified with 967 parts of water using a colloid mill. The emulsion produced contained 3 per cent of siloxane. This emulsion was employed for treating acetate rayon. One sample of the fabric was heated after treating, at a temperature of 150° C. for 20 minutes. Following this the fabric had a spray rating of 90. The fabric was next washed with soap. The fabric still had a spray rating of 90 and was free of objectionable mark-off.

## Example 2

A mixture was prepared of 24 parts by weight of product IV and 6 parts of product II. To this siloxane mixture there were then added 3 parts of hexadecyldimethylbenzylammonium chloride and 0.1049 of acetic acid. The resulting mixture was then emulsified with 967 parts of water using a colloid mill. This produced an emulsion containing 3 per cent siloxane. The emulsion was employed for treating acetate rayon. One sample of the fabric was heated after treating at a temperature of 150° C. for 5 minutes. Following this the fabric had a spray rating of 90. The fabric was next washed with soap, following which it had a spray rating of 80 to 90. It was noted that the fabric was free of objectionable mark-off.

## Example 3

A mixture was prepared of 18 parts by weight of product IV, 15 parts of water, 19 parts of toluene and 12 parts of product II. To this siloxane mixture there were then added 3 parts of hexadecyldimethylbenzylammonium chloride. The resulting mixture was then emulsified with 942 parts of water using a colloid mill. The emulsion produced contained 3 per cent of siloxane. This emulsion was employed for treating

the following fabrics for 5 and 10 minutes at 150° C. giving the spray rating indicated.

|                       | 5 min./<br>150° C. | 10 min./<br>150° C. |
|-----------------------|--------------------|---------------------|
| (1) Muslin            | 90                 | 90                  |
| (2) Plaid Twill       | 90                 | 100                 |
| (3) Acetate Sharkskin | 90                 | 100                 |

The rayon fabric was free of objectionable mark-off.

*Example 4*

A mixture was prepared of 67 parts by weight of product IV, 19 parts of water, 74 parts of methylene chloride and 67 parts of product II. To this siloxane mixture there were then added 8 parts of hexadecyldimethylbenzylammonium chloride. The resulting mixture was then emulsified with 3493 parts of water using a colloid mill. The emulsion produced contained 3 per cent of the siloxane mixture. This emulsion was employed for treating the following fabrics and the fabrics cured for 5 minutes at 150° C. resulting in the indicated spray ratings:

|                                              |        |
|----------------------------------------------|--------|
| (1) Muslin                                   | 100    |
| (2) Olive elkskin (cotton and viscose rayon) | 100    |
| (3) Wool twill                               | 90     |
| (4) Acetate sharkskin                        | 100    |
| (5) Acetate French crepe                     | 70     |
| (6) Acetate satin                            | 70     |
| (7) Acetate and rayon faille                 | 90-100 |
| (8) Viscose rayon suiting                    | 100    |

The treated fabrics had a good hand, and the rayon fabrics were free of objectionable mark-off.

*Example 5*

A mixture was prepared of 354 parts by weight of methylene chloride, 248.5 parts of water and 177 parts of product III. To this mixture there were then added 17 parts of hexadecyldimethylbenzylammonium chloride, and the mixture emulsified using a colloid mill. This emulsion was added to 154 parts of product IV. 10,000 parts of water were then added to the emulsion. The mixture was then emulsified using a colloid mill. The following fabrics were treated for 5 minutes at 150° C. after which time the fabrics had the spray ratings indicated:

|                   |     |
|-------------------|-----|
| (1) Muslin        | 80  |
| (2) Cotton twill  | 80  |
| (3) Acetate rayon | 90  |
| (4) Nylon tenting | 100 |

The fabrics all had a good hand and the rayon and nylon fabrics were free of objectionable mark-off.

*Example 6*

A solution was prepared of 194 parts by weight of toluene, 3.6 parts of product IV and 2.4 parts of product II. Acetate rayon twill fabric was coated with this solution and the fabric cured for 10 minutes at 450° F. Following this, the fabric had a spray rating of 80. The fabric had a good hand and was free of objectionable mark-off.

*Example 7*

A solution was prepared of 194 parts by weight of toluene, 2.4 parts of product IV and 3.6 parts of product II. An acetate rayon twill was coated with this solution and cured for 10 minutes at 150° C. Following this, the spray rating was 80.

The fabric was soft and was free of objectionable mark-off.

*Example 8*

5 A solution was prepared of 194 parts by weight of toluene, .78 part of product IV and 5.22 parts of product II. Acetate rayon twill was coated with this solution and cured for 10 minutes at 150° C. Following this, the spray rating of the fabric was 90. The fabric had a good hand. The fabric was free of objectionable mark-off. Following dry cleaning the fabric had a spray rating of 70.

*Example 9*

15 A mixture was prepared of 1405 parts by weight of product IV, 935 parts of product II and 1260 parts of methylene chloride. To this siloxane mixture there were then added 234 parts of hexadecyldimethylbenzylammonium chloride. The resulting mixture was then emulsified with 2016 parts of water using a colloid mill. The emulsion produced was diluted with 52,650 parts of water. This gave an emulsion containing 4 per cent of siloxane. This emulsion was employed for treating the following fabrics for 5 minutes at 25 150° C. giving the spray rating indicated:

|                       |     |
|-----------------------|-----|
| (1) Muslin            | 100 |
| (2) Cotton twill      | 100 |
| (3) Orlon             | 100 |
| (4) Nylon             | 100 |
| (5) Nylon tenting     | 100 |
| (6) Wool              | 100 |
| (7) Acetate twill     | 100 |
| (8) Acetate sharkskin | 100 |

35 All of the above fabrics had a soft hand, and the rayon, nylon and orlon fabrics were free of objectionable mark-off.

That which is claimed is:

40 1. The method of rendering organic fabrics water-repellent, which comprises wetting the fabrics with a mixture of from 20 to 70 per cent by weight of a methylpolysiloxane containing between 2 and 2.1 methyl radicals per silicon atom and having a viscosity of at least 1,000 centistokes and from 80 to 45 30 per cent of a methylhydrogenpolysiloxane containing between 1.0 and 1.5 methyl radicals and between 0.75 and 1.25 hydrogen atoms bonded to silicon per silicon atom, there being a total of 2 to 2.25 methyl radicals and hydrogen atoms per silicon atom, and heating the wetted fabrics at a 50 temperature of from 100° to 475° F. for a period of from 5 seconds to 1 hour, whereby the fabrics are rendered water-repellent.

55 2. The method of rendering organic fabrics water-repellent, which comprises wetting the fabrics with an aqueous emulsion of a mixture of from 20 to 70 per cent by weight of a methylpolysiloxane containing between 2 and 2.1 methyl radicals per silicon atom and having a viscosity of at least 1,000 centistokes and less than 100,000 centistokes, and from 80 to 60 30 per cent of a methylhydrogenpolysiloxane containing between 1.0 and 1.5 methyl radicals and between 0.75 and 1.25 hydrogen atoms bonded to silicon per silicon atom, there being a total of 2 to 2.25 total methyl radicals and hydrogen atoms bonded to silicon per silicon atom, which emulsion contains a trialkylbenzylammonium chloride as an emulsifying agent, and heating the wetted fabric at a temperature of from 100° to 475° F. for a period of from 5 seconds to 1 hour, whereby the fabrics are rendered water-repellent and the emulsifying agent is decomposed.

70 3. An organic textile fabric coated with be-

tween 1 and 5 per cent based upon the weight of the fabric of a polymerized mixture of from 20 to 70 per cent by weight of a methylpolysiloxane containing between 2 and 2.1 methyl radicals per silicon atom and having a viscosity of at least 1,000 centistokes and less than 100,000 centistokes, and from 80 to 30 per cent of a methylhydrogenpolysiloxane containing between 1.0 and 1.5 methyl radicals and between 0.75 and 1.25 hydrogen atoms bonded to silicon per silicon atom, there being a total of 2 to 2.25 methyl radicals and hydrogen atoms per silicon atom.

FIRTH L. DENNETT.

**REFERENCES CITED**

The following references are of record in the file of this patent:

UNITED STATES PATENTS

|    | Number    | Name       | Date           |
|----|-----------|------------|----------------|
| 5  | 2,258,218 | Rochow     | Oct. 7, 1941   |
|    | 2,285,562 | Britton    | June 9, 1942   |
|    | 2,306,222 | Patnode    | Dec. 22, 1942  |
|    | 2,314,111 | Tucker     | Mar. 16, 1943  |
|    | 2,384,384 | McGregor   | Sept. 4, 1945  |
| 10 | 2,386,259 | Morton     | Oct. 9, 1945   |
|    | 2,390,370 | Hyde       | Dec. 4, 1945   |
|    | 2,392,805 | Biefeld    | Jan. 15, 1946  |
|    | 2,395,070 | Sarbach    | Feb. 19, 1946  |
|    | 2,397,451 | West       | Mar. 26, 1946  |
|    | 2,408,822 | Tanis, Jr. | Oct. 8, 1946   |
|    | 2,439,689 | Hyde       | Apr. 13, 1948  |
| 15 | 2,449,572 | Welsh      | Sept. 21, 1948 |
|    | 2,491,843 | Wilcox     | Dec. 20, 1949  |
|    | 2,494,920 | Warrick    | Jan. 17, 1950  |
|    | 2,500,842 | MacKenzie  | Mar. 14, 1950  |
|    | 2,528,554 | Rust       | Nov. 7, 1950   |